

A. P. DERBY & J. H. DARGIE,  
PROCESS FOR THE TREATMENT OF WOOD,  
APPLICATION FILED AUG. 7, 1913.

1,186,555

Patented June 13, 1916.



Witnesses

R. H. Tolman.  
Leopold Comberbach.

Inventors  
Ashton P. Derby.  
James H. Dargie.

By Rufus B. Fowler

Attorney

# UNITED STATES PATENT OFFICE.

ASHTON P. DERBY AND JAMES H. DARGIE, OF GARDNER, MASSACHUSETTS, ASSIGNEES  
TO P. DERBY AND COMPANY, INC., OF GARDNER, MASSACHUSETTS, A CORPORATION  
OF MASSACHUSETTS.

## PROCESS FOR THE TREATMENT OF WOOD

1,186,555.

Specification of Letters Patent. Patented June 13, 1916.

Application filed August 7, 1913. Serial No. 733,517.

To all whom it may concern:

Be it known that we, ASHTON P. DERBY and JAMES H. DARGIE, both citizens of the United States, residing at Gardner, in the county of Worcester and Commonwealth of Massachusetts, have invented a new and useful Process for the Treatment of Wood, of which the following is a specification, accompanied by a drawing forming a part 10 of the same.

Our invention relates to an improved method of treating wood by which the sap is removed and the wood rendered suitable for immediate use, thereby avoiding the 15 long delay incident to the commonly practised method of seasoning wood by atmospheric exposure.

In carrying out our improved process into effect we employ an apparatus shown partly 20 in sectional view in the accompanying drawing, comprising a chamber 1 in which the material to be treated may be inclosed. Within the chamber 1 is a track 2 upon which a truck 3 may be moved, carrying 25 the material to be treated, which in the present instance is represented as a pile of boards 4 spaced apart, as shown at 5, 5, to allow the introduction of steam around each individual piece. One side of the receptacle 30 inclosing the chamber 1 is provided with a door 6 closing against a gasket 7 which renders the chamber air tight.

Leading from a source of steam supply under pressure is a pipe 8 entering the chamber 1 and provided with a valve 9 by which the supply of steam to the chamber 1 may be regulated. From the chamber 1 we conduct a pipe 10 leading to an air pump 11 having a discharge nozzle 12 and operated through 40 a piston rod 13 and rotating eccentric 14 which is carried upon a shaft 15 and driven from any suitable source of power by means of a belt pulley 16. The wood to be treated is loaded upon the truck 3, each piece being 45 suitably spaced from its neighbor and the truck placed upon the track 2. The door 6 is then closed, hermetically closing the chamber 1. Steam is admitted through the pipe for the space of from thirty to forty 50 five minutes at a pressure of about fifty pounds. At the end of this period the sup-

ply of steam is shut off by the valve 9 and the air pump 11 put in operation until the steam and air contained in the chamber 1 is substantially exhausted. The wood is 55 then allowed to remain in the vacuum thus produced for a short period, depending somewhat upon the nature of the wood, usually about one half hour for each inch in thickness of the wood. 60

During the above described process we admit steam under pressure through a pipe 17 to a radiator 18 inclosed in the chamber 1 and preferably provided with the usual automatic air valve, for the purpose of maintaining a temperature in the chamber 1 sufficient to prevent the substantial condensation of steam and to accomplish the more thorough evaporation of moisture while the wood remains in the vacuum. The lumber 70 is then removed from the chamber 1 thoroughly seasoned or deprived of its sap, and in proper condition for immediate use either with or without further kiln drying, according to the purpose for which it is to 75 be employed.

If the wood is to be used for cabinet work, furniture, or interior finish, it should be kiln dried by the method now commonly practised by the application of dry heat immediately before such use.

We claim,

The within described process of treating wood, consisting in inclosing the wood in a hermetically sealed chamber, subjecting the 85 wood in said chamber to the action of steam under pressure for a predetermined period, maintaining during said period a temperature in said chamber sufficient to prevent the condensation of steam, exhausting the air 90 and steam from said chamber at the end of said period, and subjecting said wood to the action of heat during the predetermined time which it remains in the vacuum thus produced. 95

Dated this fourth day of August, 1913.

ASHTON P. DERBY.  
JAMES H. DARGIE.

Witnesses:

MADALENE P. BLACK,  
AMASA B. BRYANT.